# EUROPEAN PATENT SPECIFICATION

(11) **EP 2 331 340 B1**
(45) Date of publication and mention of the grant of the patent: **11.07.2012**
(21) Application number: 08788780.8
(22) Date of filing: 10.09.2008
(51) Int. Cl.: B41M 3/14, B41M 5/26, B41M 5/28, B41M 5/30, B41M 5/42

(54) **LASER IMAGING AND ITS USE IN SECURITY APPLICATIONS**
LASERABBILDUNG UND IHRE VERWENDUNG IN SICHERHEITSANWENDUNGEN
MARQUAGE LASER ET SON UTILISATION DANS DES APPLICATIONS DE SÉCURITÉ

(43) Date of publication of application: 15.06.2011
(73) Proprietor: DataLase Ltd, Widnes Cheshire WA8 8FW (GB)
(72) Inventor: JARVIS, Anthony N., Widnes Cheshire WA8 8FW (GB); WYRES, Christopher Anthony, Widnes Cheshire WA8 8FW (GB)
(74) Representative: Creek, Isobel Clare
(86) International application number: PCT/GB2008/050811
(87) International publication number: WO 2010/029276

(56) References cited:
- EP-A- 0 987 121
- DE-A- 10 115 949
- JP-A- 2 153 782
- JP-A- 61 248 785

## Description

### Field of the Invention

This invention relates to laser-imaging and its use in security applications.

### Background of the Invention

There is a growing demand for marking articles with covert indicia in order to prevent counterfeiting, forgeries and ID theft. This includes official documents such as passports, identity cards, banknotes, high value branded goods, pharmaceutical compositions, foodstuffs and pin numbers or other access codes.

US5719939 discloses the creation of a unique pattern of overlying individual fibers which are embedded in a transparent base material, such that the fibers form differing geometrical configurations which are optically scannable through a surface of the transparent base material. This system suffers from several drawbacks; notably, it cannot be performed on a rapidly moving production line.

WO98/40224 describes a method of marking glassy thermoplastic polymeric material with a sub-surface mark. Laser radiation is directed at the surface of the material and this produces localised stresses within the material which cannot be detected at the surface by the naked eye, but which are capable of being rendered visible under polarised light.

However, in all of these techniques the indicia are placed overtly on the article. Indicia that cannot be seen with the human eye are even more difficult to reproduce than those that are visible.

EP0987121 discloses a method of forming an invisible bar code indicium on an article that comprises an outer opaque, black layer and an inner, laser-imageable layer, the method comprising irradiating the article with a laser at 248 nm, whereby the laser radiation passes through the opaque layer and causes the laser-imageable leuco dye photosensitive layer to change colour.

Similar disclosures are found in JP61248785, JP02153782 and DE10115949.

### Summary of the Invention

In a first aspect, the present invention is a method of forming an invisible indicium on an article that comprises an outer opaque layer and an inner laser-imageable layer, which comprises irradiating the article with a laser, whereby the laser radiation passes through the opaque layer and causes the laser-imageable layer to change colour; wherein the laser-imageable layer comprises a colour-former which is a metal oxyanion or a diacetylene.

In a second aspect, the present invention is an article comprising an outer opaque layer and an inner layer comprising or coated with a laser-imageable composition and in or on which images have been formed, wherein the laser imageable layer comprises a colour-former which is a metal oxyanion or a diacetylene.

The outer layer is generally opaque to the human eye but transparent to laser radiation. The indicium is produced in the inner, laser-imageable layer, but this cannot be seen through the outer, human eye-opaque layer.

Laser imaging/marking is particularly advantageous for this application, as it allows infinitely variable information to be applied to an article.

### Brief Description of the Drawings

The accompanying drawing (Figure 1) is a schematic representation of an embodiment of the invention.

### Description of Preferred Embodiments

A laser-imageable composition utilised in this invention comprises any substance or combination of substances which change appearance or absorption profile when irradiated by a laser. The laser-imageable composition can be included within the article, such as a moulded plastic article made using a masterbatch technique, or added to paper during manufacture, or applied directly to the article such as via a spray, or applied to the article as part of a coating application using a printing technique.

Preferred examples of laser-imageable compositions that form part of the present invention are disclosed in WO02/068205, WO02/074548, WO04/043704, WO2005/012442, W02005/068207, W02006/018640, WO2006/051309, W02006/129086, W02006/129078, W02007/045912 and WO2007/063339. Examples can also be found in WO2006/063165, US2007032569, US7169471, US5413629, US5955224, W02006/052843, W02005/026247 and WO2005/047010. Particularly preferred examples of constituents of the laser-imageable compositions are ammonium octamolybdate (AOM), leuco dyes, carbazoles, diacetylenes, and dehydration agents with hydroxyl-containing compounds.

When employing a near-infrared laser, it is desirable to incorporate a near-infrared absorbing substance in the formulation. Examples include near infrared absorbing compounds such as those that have an absorbance maximum similar to the wavelength of the near infrared radiation employed and preferably have little or no visible colour. Suitable examples include copper compounds such as copper (II) hydroxyl phosphate (CHP) supplied as Fabulase 322 by Budenheim, mixed metal oxide compounds particularly non-stoichiometric reduced versions such as reduced indium tin oxide (such as Degussa's AdNano products) or reduced antimony tin oxide, organic polymers such as the conductive polymer product Baytron^{®} P supplied by HC Starck, coated inorganic particles including antimony tin oxide coated micas and the Lazerflair and Iriodin products supplied by Merck, and near infrared absorbing organic molecules, known to those skilled in the art as NIR dyes/pigments. Types of NIR dyes/pigments than can be used comprise, but are not limited to: families of metallo-porphyrins, metallo-thiolenes and polythiolenes, metallophthalocyanines, aza-variants of these, annellated variants of these, pyrylium salts, squaryliums, croconiums, amminiums, diimoniums, cyanines and indolenine cyanines.

Examples of organic compounds that can be used in the present invention are taught in US6911262, and are given in "Developments in the Chemistry and Technology of Organic dyes", J Griffiths (ed), Oxford: Blackwell Scientific, 1984, and "Infrared Absorbing Dyes", M Matsuoka (ed), New York: Plenum Press, 1990. Further examples of the NIR dyes or pigments of the present invention can be found in the Epolight™ series supplied by Epolin, Newark, NJ, USA; the ADS series supplied by American Dye Source Inc, Quebec, Canada; the SDA and SDB series supplied by HW Sands, Jupiter, FL, USA; the Lumogen™ series supplied by BASF, Germany, particularly Lumogen™ IR765, IR788 and IR1055; and the Pro-Jet™ series of dyes supplied by FujiFilm Imaging Colorants, Blackley, Manchester, UK, particularly Pro-Jet™ 830NP, 900NP, 825LDI and 830LDI and the Filtron™ products supplied by Gentex Corp of Carbondale, PA.

Other energy absorbing components include UV absorbers, visible dyes and pigments, and agents to absorb 10.6 microns energy such as inorganic particles such as calcium salts such as the phosphate, hydroxyphosphate and carbonate, talc, clays, micas, titanium dioxide, molybdates such as ammonium octamolybdate and the like.

A laser imageable layer may also comprise an acid or base generating agent. The acid generating agent can be a thermal or photo acid generating agent. Examples include 'onium' type compounds particularly sulphonium and iodonium agents such as triarylsulphonium hexafluoroantimonate salts in propylene carbonate at 50%.

Each indicium can be comprised of 2-dimensional shapes such as lines, dots, circles, elipses, polygons etc. or combinations thereof. The shapes can be geometric or non-geometric. The shapes can be monochrome, multicoloured or combinations of both. The indicium can be any indicium known to those skilled in the art. Examples include human or machine-readable code, such as symbols, barcodes or matrix codes.

The invention is particularly suitable for the generation of machine-readable codes such as barcodes, as this allows the articles to be automatically identified and tracked throughout their lifecycle down to an individual level. This then provides the basis of a 'track and trace' system for the articles.

A definition of a barcode and other symbologies that form part of the present invention can be found at http://en.wikipedia.org/wiki/Barcode.

A laser-imageable composition can be incorporated into a structure beneath a substrate which is opaque to visible light but transparent to NIR light. This allows a coloured indicium of the present invention to be created in the laser-imageable composition using a NIR laser that is not visible to the eye, but can be detected using a NIR scanner such as a camera.

The profile of the laser beam can be tailored to any given shape, size or energy distribution, using appropriate beam-shaping optics.

The laser can have an emission wavelength in the region 200 nm - 20 µm. Preferred lasers are carbon dioxide lasers, NIR lasers, visible band lasers and UV lasers. Particularly preferred lasers are NIR lasers, such as DPSS lasers, fibre lasers, diode lasers and laser diode arrays. Both pulsed and continuous wave lasers can be used. Non-coherent and broadband radiation can also be used. In this case images can be produced using a mask.

The article can be any substrate, such as glass, film, paper, plastics, wood, foodstuffs, pharmaceuticals or any substance that a laser-sensitive agent can be incorporated into. The laser-sensitive agent can also be formulated into an ink, paint or lacquer, and then applied to the substrate using any suitable technique. Particularly preferred substrates are those that can be used to make banknotes, the outer shell of pharmaceutical tablets, excise stamps, ID and high value documents such as passports and driving licenses, the packaging of consumer goods, and those used to divulge pin numbers and access codes.

The present invention is the creation of indicia on an article, using a laser-imageable composition whereby a laser causes the composition to change colour, through a layer opaque to the human eye but transparent to laser radiation. This is illustrated schematically in the accompanying drawing (Figure 1).

Such a system is useful in security applications where indicia such as barcodes and the like, and other information such as human-readable pin numbers and text, can be created on an article but cannot be read or seen by the human eye due to the overlying opaque layer. However, such indicia and information can be read through the overlying opaque layer using a suitable scanning device. If desired, the opaque layer may be removable; removal will reveal the indicia and information on the article to a suitable scanning device or to the human eye.

The laser-imageable layer can be any laser-imageable layer as described in the present invention. The opaque layer is preferably opaque to the human eye but transparent to laser radiation. A particularly preferred system is that based on a near-infrared (NIR) laser comprising a NIR-transparent but human eye-opaque overlayer, and a NIR-imageable inner layer on the article to be marked. A NIR-transparent but human eye-opaque overlayer can be created by coating a substrate substantially transparent to NIR radiation such as clear PET or clear BOPP with a coating of a ink opaque to the human eye but transparent to NIR radiation. A particularly preferred ink is one of the same colour as the indicia/information created on the laser-imageable inner layer and transparent to NIR radiation. Inks comprising perylene pigments are particularly preferred due to their high degree of NIR-transparency. C.I. Pigment Black 31 is a suitable example of such an ink. The human eye opaque/laser radiation transparent agent can also be formulated directly into the bulk of the layer as well as coated on to its surface. This could be done by extruding a film comprising the agent mixed into the polymer that comprises the film.

The following Examples illustrate the invention.

### Chemicals:

Paranol T-6320 (aqueous acrylic-urethane resin) - ex. Para-Chem. Octafoam E-235 (defoamer) - ex. Octel.
Yamada ETAC (black/green leuco dye) - ex. Yamada Chemical Co. Ltd. Benzyl p-hydroxybenzoate - supplied by Acros.
Copper (II) hydroxyl phosphate (CHP) - was supplied by Budenheim as Fabulase 322.
*N*-ethyl carbazole - supplied by Aldrich.
Nitrocellulose DLX3-5 - supplied by Nobel Enterprises nitrocellulose. Elvacite 2028 (acrylic binder) - supplied by Lucite International.
Cyracure 6974 (a photoacid generator) - supplied by Dow Chemicals. 10,12-pentacosadiynoic acid - supplied by Aldrich.
AdNano reduced ITO powder was supplied by Degussa.
Paliogen Black S 0084, Cl Pigment Black 31, was supplied by BASF.

### Substrates:

Natural top liner paper
White 50 µm PET film - supplied by HiFi.
Clear 50 µm PET film - supplied by HiFi.

### Lasers:

A 30W Videojet CO₂ laser connected to a galvanometer scanning head and controlled by an IBM-compatible PC and software.

A 10W SPI 1550nm fibre laser connected to a galvanometer scanning head and controlled by an IBM-compatible PC and software.

A 10W SPI 1066nm fibre laser connected to a galvanometer scanning head and controlled by an IBM-compatible PC and software.

A 3W Avia-Coherent 266nm, diode-pumped, all-solid state, Q-switched laser connected to a galvanometer scanning head and controlled by an IBM compatible PC and software.

### Example A -Outer Opaque Black Layer

The following ink formulation was prepared:
Nitrocellulose DLX3-5 dissolved in 3:1 ethanol/ethyl acetate (15%) = 90 g
Paliogen Black S 0084 = 10 g

Mill using an Eiger-Torrance 50ml bead mill for 15 minutes and coat on to clear PET film using a RK Proofer Printer fitted with a K-3 bar (to give about 8gsm).

### Example 1

The following ink formulation was prepared:

| | |
|---|---|
| Paranol T-6320 | = 44 g |
| Octafoam E-235 | = 1 g |
| AOM | = 55 g |

The ink was prepared using a high speed Silverson mixer for 15 minutes prior to its application to the substrate.

### Example 2

The following ink formulation was prepared:

| | |
|---|---|
| Paranol T-6320 | = 44 g |
| Octafoam E-235 | = 1 g |
| AOM | = 35 g |
| CHP | = 20 g |

The ink was milled using an Eiger-Torrance bead mill (50 ml) for 15 minutes prior to its application to the substrate.

### Example 3

The following ink formulation was prepared:

| | |
|---|---|
| Paranol T-6320 | = 59 g |
| Octafoam E-235 | = 1 g |
| AOM | = 35 g |
| AdNano reduced ITO powder | = 5 g |

The ink was milled using an Eiger-Torrance bead mill (50 ml) for 15 minutes prior to its application to the substrate.

### Example 4 - comparative

The following ink formulation was prepared:

| | |
|---|---|
| Paranol T-6320 | = 79 g |
| Octafoam E-235 | = 1 g |
| Yamada ETAC | = 5 g |
| BHB | = 15 g |

The ink was prepared using a high speed Silverson mixer for 15 minutes prior to its application to the substrate.

### Example 5 - Comparative

The following ink formulation was prepared:

| | |
|---|---|
| Paranol T-6320 | = 59 g |
| Octafoam E-235 | = 1 g |
| Yamada ETAC | = 5 g |
| BHB | = 15g |
| CHP | = 20 g |

The ink was milled using an Eiger-Torrance bead mill (50 ml) for 15 minutes prior to its application to the substrate.

### Example 6 - Comparative

The following ink formulation was prepared:

| | |
|---|---|
| Nitrocellulose DLX3-5 15% in MEK | = 80 g |
| *N*-Ethyl carbazole | = 5 g |
| Cyracure 6974 | = 15 g |

The ink was prepared by stirring the above formulation for 2 hours prior to its application to the substrate.

### Example 7

The following ink formulation was prepared:

| | |
|---|---|
| Elvacite 2028 15% in MEK | = 80 g |
| 10,12-pentacosadiynoic acid | = 5 g |
| Cyracure 6974 | = 15g |

The ink was prepared by stirring the above formulation for 2 hours prior to its application to the substrate.

Each formulation prepared in Examples 1 to 7 was coated on to natural top liner and white PET film using an RK Proofer Printer fitted with a K-3 bar to give a coat weight of approximately 6 to 8gsm. The coated substrates were then covered by the opaque black layer prepared using the Paliogen Black ink. The bi-layer substrate composition was then laser imaged through the outer opaque black layer.

The following laser/substrate combinations were used:
Examples 1 and 4 were imaged with the CO₂ laser.
Examples 2 and 5 were imaged using the 1066nm NIR fibre laser. Example 3 was imaged using the 1550nm fibre NIR laser.
Examples 6 and 7 were imaged using the 266nm UV laser.

In each case a machine readable code and a human readable 4 digit pin number were imaged.

After imaging it was not possible to see the image in the inner imageable layer underneath the outer opaque black layer. However, removing the outer opaque black layer revealed the inner imaged layer.

## Claims

1. A method of forming an invisible indicium on an article that comprises an outer opaque layer and an inner laser-imageable layer, which comprises irradiating the article with a laser, whereby the laser radiation passes through the opaque layer and causes the laser-imageable layer to change colour; wherein the laser imageable layer comprises a colour former which is a metal oxyanion or a diacetylene.

2. A method as claimed in claim 1, wherein the opaque layer is opaque to the human eye, preferably wherein the opaque layer is black.

3. A method as claimed in claim 2, wherein the opaque layer comprises a perylene colorant.

4. A method as claimed in any preceding claim, wherein a laser-imageable composition is provided within an article that comprises the inner layer, or forms the inner layer by being coated on to an article.

5. A method as claimed in any preceding claim, wherein the laser has an emission wavelength in the region 200 nm to 20 microns.

6. A method as claimed in claim 5, wherein the laser is a near infrared laser with an emission wavelength in the region 700 nm to 2500nm, preferably where the near infrared laser is a fibre, diode or diode array laser.

7. A method as claimed in any preceding claim, wherein the indicium is selected from one or more of human readable text, devices, numbers or lines, dots, circles, polygons or ellipses.

8. A method as claimed in any preceding claim, which comprises forming a plurality of indicia which each comprise 2-dimensional shapes, and the indicia are distinct for distinct articles.

9. A method as claimed in any preceding claim wherein the outer layer is opaque to the human eye but transparent to laser radiation with an emission wavelength in the region 700 to 2500nm, and the inner layer is imageable by said 700 to 2500nm laser radiation.

10. A method according to any preceding claim, wherein the metal oxyanion is a molybdate such as ammonium octamolybdate.

11. A method according to any preceding claim, wherein the inner layer comprises a near-infrared absorbing additive.

12. A method according to claim 11, wherein the near-infrared absorbing additive is copper (II) hydroxide phosphate, a non-stoichiometric mixed metal oxide such as reduced indium tin oxide, a conductive polymer or an organic dye/pigment.

13. A method according to any preceding claim, wherein the imageable layer further comprises an acid generating agent.

14. An article comprising an outer opaque layer and an inner layer comprising or coated with a laser-imageable composition and in or on which images have been formed, wherein the laser imageable layer comprises a colour former which is a metal oxyanion or a diacetylene.

15. A method for checking the authenticity of an article as claimed in claim 14, which comprises scanning the article and determining the presence of the images.

## Patentansprüche

1. Verfahren zum Bilden eines unsichtbaren Zeichens auf einem Artikel, der eine äußere opake Schicht und eine innere mit Laser bebilderbare Schicht umfasst, umfassend das Bestrahlen des Artikels mit einem Laser, wodurch die Laserstrahlung durch die opake Schicht gelangt und bewirkt, dass die mit Laser bebilderbare Schicht die Farbe ändert; wobei die mit Laser bebilderbare Schicht einen Farbbildner umfasst, bei dem es sich um ein Metall-Oxyanion oder ein Diacetylen handelt.

2. Verfahren nach Anspruch 1, wobei die opake Schicht für das menschliche Auge opak ist, vorzugsweise, wobei die opake Schicht schwarz ist.

3. Verfahren nach Anspruch 2, wobei die opake Schicht einen Perylenfarbstoff umfasst.

4. Verfahren nach einem der vorangehenden Ansprüche, wobei eine mit Laser bebilderbare Zusammensetzung in einem Artikel vorgesehen ist, der die innere Schicht umfasst oder die innere Schicht bildet, indem er auf einen Artikel beschichtet ist.

5. Verfahren nach einem der vorangehenden Ansprüche, wobei der Laser eine Emissionswellenlänge im Bereich 200 nm bis 20 Mikrometer aufweist.

6. Verfahren nach Anspruch 5, wobei es sich bei dem Laser um einen Nahinfrarotlaser mit einer Emissionswellenlänge im Bereich 700 nm bis 2500 nm handelt, vorzugsweise, wobei es sich bei dem Nahinfrarotlaser um einen Faser-, Dioden- oder Diodenarray-Laser handelt.

7. Verfahren nach einem der vorangehenden Ansprüche, wobei das Zeichen ausgewählt wird aus einem oder mehreren von von Menschen lesbarem Text, Devisen, Zahlen oder Linien, Punkten, Kreisen, Polygonen oder Ellipsen.

8. Verfahren nach einem der vorangehenden Ansprüche, umfassend das Bilden von mehreren Zeichen, die jeweils zweidimensionale Formen umfassen und wobei die Zeichen für verschiedene Artikel verschieden sind.

9. Verfahren nach einem der vorangehenden Ansprüche, wobei die äußere Schicht für das menschliche Auge opak ist aber für Laserstrahlung mit einer Emissionswellenlänge im Bereich 700 bis 2500 nm transparent ist und die innere Schicht von der genannten Laserstrahlung mit 700 bis 2500 nm bebilderbar ist.

10. Verfahren nach einem der vorangehenden Ansprüche, wobei es sich bei dem Metall-Oxyanion um ein Molybdat wie etwa Ammonium-Oktamolybdat handelt.

11. Verfahren nach einem der vorangehenden Ansprüche, wobei die innere Schicht ein nahinfrarotabsorbierendes Additiv umfasst.

12. Verfahren nach Anspruch 11, wobei es sich bei dem nahinfrarotabsorbierenden Additiv um Kupfer (II) Hydroxidphosphat, ein nicht stöchiometrisches gemischtes Metalloxid wie etwa reduziertes Indiumzinnoxid, ein leitfähiges Polymer oder ein organisches Färbemittel/Pigment handelt.

13. Verfahren nach einem der vorangehenden Ansprüche, wobei die bebilderbare Schicht weiter ein säureerzeugendes Mittel umfasst.

14. Artikel, umfassend eine äußere opake Schicht und eine innere Schicht, die eine mit Laser bebilderbare Zusammensetzung umfasst oder damit beschichtet ist und in oder auf der Bilder gebildet wurden, wobei die mit Laser bebilderbare Schicht einen Farbbildner umfasst, bei dem es sich um ein Metall-Oxyanion oder ein Diacetylen handelt.

15. Verfahren zum Prüfen der Echtheit eines Artikels nach Anspruch 14, umfassend das Abtasten des Artikels und das Bestimmen der Anwesenheit der Bilder.

## Revendications

1. Procédé permettant de former un repère invisible sur un article qui comporte une couche extérieure opaque et une couche intérieure permettant la formation d'images au laser, qui comporte l'étape consistant à irradier l'article au moyen d'un laser, ce par quoi le rayonnement laser traverse la couche opaque et entraîne la couche permettant la formation d'images au laser à changer de couleur ; dans lequel la couche permettant la formation d'images au laser comporte une substance chromogène qui est un oxyanion de métal ou un diacétylène.

2. Procédé selon la revendication 1, dans lequel la couche opaque est opaque vis-à-vis de l'oeil humain, de préférence dans lequel la couche opaque est noire.

3. Procédé selon la revendication 2, dans lequel la couche opaque comporte un colorant pérylène.

4. Procédé selon l'une quelconque des revendications précédentes, dans lequel une composition permettant la formation d'images au laser est mise en oeuvre à l'intérieur d'un article qui comporte la couche intérieure, ou forme la couche intérieure en étant appliquée sur un article.

5. Procédé selon l'une quelconque des revendications précédentes, dans lequel le laser a une longueur d'onde d'émission de l'ordre de 200 nm à 20 microns.

6. Procédé selon la revendication 5, dans lequel le laser est un laser infrarouge proche ayant une longueur d'onde d'émission de l'ordre de 700 nm à 2500 nm, de préférence quand le laser infrarouge proche est un laser à fibre, à diode ou à réseau de diodes.

7. Procédé selon l'une quelconque des revendications précédentes, dans lequel le repère est sélectionné parmi un ou plusieurs entre du texte, des dispositifs, des nombres ou des lignes, des points, des cercles, des polygones ou des ellipses que peut lire l'utilisateur.

8. Procédé selon l'une quelconque des revendications précédentes, qui comporte une étape consistant à former une pluralité de repères qui comportent chacun des formes bidimensionnelles, et les repères étant distincts pour des articles distincts.

9. Procédé selon l'une quelconque des revendications précédentes, dans lequel la couche extérieure est opaque vis-à-vis de l'oeil humain mais transparente par rapport au rayonnement laser à une longueur d'onde d'émission de l'ordre de 700 nm à 2500 nm, et la couche intérieure permet la formation d'images par ledit rayonnement laser de 700 à 2500 nm.

10. Procédé selon l'une quelconque des revendications précédentes, dans lequel l'oxyanion de métal est un molybdène tel un octamolybdène d'ammonium.

11. Procédé selon l'une quelconque des revendications précédentes, dans lequel la couche intérieure comporte un additif absorbant l'infrarouge proche.

12. Procédé selon la revendication 11, dans lequel l'additif absorbant l'infrarouge proche est un phosphate d'hydroxyde de cuivre (II), un oxyde métallique mixte non stoechiométrique tel de l'oxyde d'étain et d'indium à réduction, un polymère conducteur ou un colorant/pigment organique.

13. Procédé selon l'une quelconque des revendications précédentes, dans lequel la couche permettant la formation d'images comporte par ailleurs un agent acidogène.

14. Article comportant une couche extérieure opaque et une couche intérieure comportant ou enduite d'une composition permettant la formation d'images au laser et dans ou sur laquelle des images ont été formées, dans lequel la couche permettant la formation d'images au laser comporte une substance chromogène qui est un oxyanion de métal ou un diacétylène.

15. Procédé permettant de vérifier l'authenticité d'un article selon la revendication 14, qui comporte l'étape consistant à examiner l'article par balayage pour déterminer la présence des images.
